

## UNITED STATES PATENT OFFICE

2,029,971

MIXED CELLULOSE ACETATE-NATURAL  
SILK FABRICS

Leo Wallerstein, Rowland A. Gale, and Thomas G. Hawley, Jr., New York, N. Y., assignors to Wallerstein Company, Inc., a corporation of New York

No Drawing. Application April 26, 1934,  
Serial No. 722,507

## 1 Claim. (Cl. 139—420)

The present invention relates to silk fabrics and it particularly relates to improved novel fabrics composed of cellulose ester yarns and natural silk yarns.

It has been possible in the last several years to make high quality yarns from cellulose esters and ethers, and particularly from cellulose acetate. For many purposes it has been found desirable to combine these cellulose esters or cellulose acetate yarns, fibres, and materials with natural silk, particularly in the manufacture of chiffon or transparent velvets.

In forming these transparent velvets, the natural silk is usually employed in gum, that is, with the strands or fibres of the natural silk being encased or coated with the gum and after the fabric is formed it is necessary to treat the fabric so as to remove this gum.

The degumming operation as a rule necessitates the employment of boiling solutions of high alkalinity containing soap. When such relatively high temperatures and alkalinites are employed, to degum the material silk contained in fabrics consisting of mixed cellulose acetate and natural silk in gum, the cellulose acetate frequently decreases in quality and is otherwise disadvantageously affected by the degumming solution.

For example, in some instances the cellulose acetate strands or fibres tend to melt or soften, particularly at temperatures of about 180° F. and above. In the case of velvets containing a cellulose acetate, an undesirable matting of the pile results from the treatment at high temperatures.

Also at about the same temperature under the alkaline conditions of the bath, the lustrous type of cellulose acetate would tend to be delustered, which was particularly objectionable in the case of many fabrics, where the cellulose acetate was primarily utilized because of its high luster.

In addition at such alkalinites and temperatures on prolonged treatment, the cellulose acetate would also tend to saponify, thereby undergoing a chemical change which alters its dyeing affinity. This change in dyeing affinity is objectionable for three reasons. It may become impossible to obtain proper cross dyeing effects. It may be necessary to employ much higher concentrates of dyestuff to obtain a given depth of shade, or it may be necessary to use an entirely different dyestuff. The dyeing affinity of all fibres

may not be changed, the same amounting giving rise to unevenness on dyeing.

For example, such a partly saponified cellulose acetate would tend to take up much greater quantities of dyes and other finishing compounds and was much less susceptible to careful control.

An object of the invention is to provide mixed cellulose acetate natural silk fabrics which may be most satisfactorily degummed under such conditions so as not to disadvantageously affect the cellulose acetate and particularly so as not to cause undesirable melting, delustering, and/or partial saponification of such cellulose acetate.

Other objects will appear during the course of the following specification.

According to the preferred embodiment of the present invention, it has been found desirable to prepare the natural silk, yarn or fibres, which are to be combined with the cellulose acetate fibres, so that the gum or bast upon such natural silk fibres may be most readily removed therefrom by relatively mild degumming operations which will only require such temperatures and alkalinites so as not to disadvantageously affect the desired qualities of the cellulose acetate material.

According to the present invention, it has been found most suitable and desirable to resort to an impregnation of the natural silk in gum before twisting, knitting, and/or weaving, said impregnation being performed with a proteolytic enzyme preparation under such conditions as not to degum the yarn and also as to leave the silk in such a condition that it may be satisfactorily handled.

Among the preferred impregnating materials are liquid baths containing proteolytic enzyme preparations, such as those derived from the growth of certain types of bacteria, fungi, and also plant enzymes, such as papain.

In the preferred procedure, the natural silk and yarn in skein form is soaked in a bath of a temperature below 50° C., said bath containing in solution or suspension, the proteolytic enzyme preparation, and also various suitable soaps and/or oils.

The natural silk, skein, or yarn, may be suspended in a soaking bath for a sufficient length of time to assure that the enzyme preparation and the other ingredients have thoroughly penetrated the raw silk fibres, and at all times the

temperature and the pH should be so maintained that substantially no degumming action results.

The details of this soaking and impregnating operations are fully set forth in the copending 5 application, of which the present application is a continuation in part, the impregnation and soaking constituting no part of the present invention. After the silk has been impregnated in this manner without any substantial visible effect upon the gum, silk may be processed by 10 winding and twisting and it may be subsequently woven alone or with other materials.

*Example 1—Silk and cellulose acetate velvet*

15 The ground warp and filling of the fabric are made of natural silk which has been suitably treated with proteolytic enzymes. The treated silk is made into threads of about 42 denier 20 twisted about 65 turns per inch. The pile warp is made of cellulose acetate which has been twisted.

The natural silk threads which have been prepared from the enzyme treated silk are treated 25 with water, for the purpose of setting the twist. After drying, the threads are woven together to make the fabric.

Degumming of the fabric is accomplished by 30 immersing in a solution of soap of from 0.25 to 5% concentration. One half of the soap may be substituted with anhydrous sodium sulfite. Temperatures varying from 110° F. to 180° F. may be used for this treatment. A gradually rising temperature may also be employed. The time required for the treatment is usually about two 35 hours. Following this treatment, the fabric is rinsed either in water or a fresh soap solution.

The degumming action in this case results from the combined actions of the enzyme and the 40 soap or sodium sulfite. The enzyme may be said to activate the soap in a manner which enables the soap to dissolve the gum at tempera-

tures much lower than would otherwise be possible.

*Example 2—Silk-cellulose acetate crepe satin*

The warp consists of silk threads of cellulose 5 acetate having only a very slight twist.

The filling is made of 5 thread Japan silk twisted 45 turns per inch, the silk in which prior to throwing has been treated with proteolytic enzymes. The threads so prepared are treated 10 with steam to set the twist. In this case the high temperature of the steam destroys all or part of the enzyme remaining and the subsequent degumming is therefore not dependent upon further enzymic action.

15 The fabric is degummed by immersing it in soap solution from 2 to 5% concentration at a temperature of 160 to 185° F. The time required is about 2 hours.

If ordinary silk had been used instead of the 20 specially prepared enzyme silk, a degumming period of about 8 hours would be required.

The present application is a continuation in 25 part of application Serial No. 606,286, filed April 19, 1932, and is similar in subject matter to co-pending applications Serial Nos. 722,504 to 722,506 and No. 722,508, all filed April 26, 1934.

The present application is particularly directed 30 to combination fabrics including cellulose acetate fibres and fibres of natural silk in gum.

What is claimed is:

A mixed cellulose acetate-natural silk fabric, 35 said natural silk being in the gum, the natural silk fibres of said fabric being impregnated with and containing a proteolytic enzyme, without degumming, said fabric being capable of being degummed at a temperature of less than 185° F. and at relatively low alkalities to prevent injury to the cellulose acetate.

LEO WALLERSTEIN.

ROWLAND A. GALE.

THOMAS G. HAWLEY, JR.

40